# EUROPEAN PATENT SPECIFICATION

(11) **EP 1 604 760 B1**
(45) Date of publication and mention of the grant of the patent: **21.02.2007**
(21) Application number: 05252858.5
(22) Date of filing: 10.05.2005
(51) Int. Cl.: B22F 1/00, B22F 1/02

(54) **A method of manufacturing a component with a cellular structure by consolidating a coated metal powder**
Verfahren zur Herstellung eines Körpers mit zellularer Struktur durch Verdichtung von beschichtetem Metallpulver
Procédé de fabrication d'un corps à structure cellulaire par densification d'une poudre métallique revêtue

(30) Priority: 12.06.2004 GB 0413135
(43) Date of publication of application: 14.12.2005
(73) Proprietor: ROLLS-ROYCE PLC, London, SW1E 6AT (GB)
(72) Inventor: Voice, Wayne Eric, West Bridgford Nottingham NG2 5JB (GB)
(74) Representative: Gunn, Michael Alan

(56) References cited:
- EP-A- 0 024 984
- GB-A- 2 157 711
- US-A- 6 024 915
- US-A- 6 162 497
- PATENT ABSTRACTS OF JAPAN vol. 016, no. 507 (M-1327), 20 October 1992 (1992-10-20) & JP 04 187704 A (DAIDO SANSO KK), 6 July 1992 (1992-07-06)

## Description

The present invention relates to a method of manufacturing a component by consolidating a metal powder.

Conventional alloys have their physical and mechanical properties improved by modifying the microstructure of the alloys by processing and heat treatment of the source ingot material, which is normally cast, though powder billet may be used.

Near net shape components are manufactured by consolidating metal powder, for example by hot isostatic pressing. In the hot isostatic pressing process a vacuum purge system is used so as to maintain the composition of the metal powder constant throughout the consolidation process. The resulting component thus has a homogeneous composition.

Accordingly the present invention seeks to provide a novel method of manufacturing a component by consolidating a metal powder in which the microstructure of the metal of the component is modified and the component has improved physical and mechanical properties.

Accordingly the present invention provides a method of manufacturing a component by consolidating a metal powder comprising the steps of:-
(a) preparing a metal powder, the metal powder comprising metal particles,
(b) depositing a coating containing at least one element on the surfaces of the metal particles of the metal powder,
(c) applying heat and pressure to consolidate the metal particles such that the at least one element of the coating on the surfaces of the metal particles partially diffuses into the metal particles and the coated metal particles are diffusion bonded together to form a cellular structure, the cellular structure comprising a framework of more highly alloyed material located at the boundaries of the diffusion bonded metal particles and the centres of the consolidated metal particles retain their original composition.

Preferably step (b) comprises oxidising the surfaces of the metal particles.

Alternatively step (b) comprises nitriding the surfaces of the metal particles.

Alternatively step (b) comprises vapour depositing a solid solution strengthening element on the surfaces of the metal particles.

Alternatively step (b) comprises coating the surfaces of the metal particles with a second metal having lower melting point than the metal particles.

Alternatively step (b) comprises coating the surfaces of the metal particles with particles of a second metal powder having a lower yield strength than the metal particles.

Preferably the metal particles have an average size of 100 micrometers. Preferably the metal particles have a maximum size of 250 micrometers.

Alternatively the size of the metal particles may be varied to vary the properties of the component.

The metal particles may be alloy particles.

The second metal may be an alloy.

The second metal particles may be alloy particles.

Preferably the metal particles are titanium alloy particles. More preferably the titanium alloy particles comprise 6wt% aluminium, 4wt% vanadium and the balance titanium, minor additions and incidental impurities.

Preferably the step a) comprises supplying the titanium alloy particles into a container, step b) comprises oxidising the titanium alloy particles, step c) comprises sealing the container and applying heat and pressure.

Preferably step b) comprises heating to a temperature of 450°C and maintaining at 450°C for 8 hours under a partial pressure of 10⁻¹ torr to oxidise the titanium alloy particles and step c) comprises hot isostatic pressing the container at a temperature of 925°C for 2 hours at a pressure of 150MPa.

Preferably the container is removed by machining or dissolving in a suitable acid. Preferably the container comprises mild steel.

The present invention also provides a component comprising consolidated metal powder, the metal powder comprising metal particles diffusion bonded together, the surfaces of the metal particles having a coating having at least one element which has partially diffused into the metal particles to form a cellular structure, the cellular structure comprising a framework of more highly alloyed material located at the boundaries of the diffusion bonded metal particles and the centres of the consolidated metal particles retain their original composition.

Preferably the coating comprising an oxide or a nitride and the at least one element is oxygen or nitrogen respectively.

Alternatively the coating comprises a solid solution strengthening element on the surfaces of the metal particles.

Alternatively the coating comprises a second metal having lower melting point than the metal particles.

Alternatively the coating comprises a second metal powder having a lower yield strength than the metal particles.

Preferably the metal particles are titanium alloy particles. More preferably the titanium alloy particles comprise 6wt% aluminium, 4wt% vanadium and the balance titanium, minor additions and incidental impurities.

Preferably the component is a gas turbine engine component.

Preferably the component is a fan blade, a part of a fan blade, a compressor blade or a casing.

The present invention will be more fully described by way of example with reference to the accompanying drawings in which:-
Figure 1 shows a component, which has been manufactured by consolidating a metal powder according to the present invention.
Figure 2 shows a further component, which has been manufactured by consolidating a metal powder according to the present invention.
Figure 3 shows an enlarged cross-sectional view through a portion of the metal powder before the start of the manufacturing process according to the present invention.
Figure 4 shows an enlarged cross-sectional view through a portion of the metal powder at a first stage of the manufacturing process according to the present invention.
Figure 5 shows an enlarged cross-sectional view through a portion of the metal powder at the end of the manufacturing process according to the present invention.

A component 10, in this example a casing, is shown in figure 1 and a further component 20, in this example a fan blade, is shown in figure 2 are manufactured by consolidating a metal powder according to the present invention.

The present invention uses a metal powder consolidation process to produce a cellular structure into a component 10 or 20 in which the normal alloy composition is held within a framework of interstitial alloy or solid solution strengthened alloy.

The method of manufacturing a component 10, or 20, by consolidating a metal powder comprises preparing a metal powder, the metal powder comprising metal particles 30. The metal particles ideally should have a narrow particle size, diameter, range, although this is not essential. For example the metal particles 30 have an average size of 100 micrometers and the metal particles 30 have a maximum size of 250 micrometers. A coating 32 containing at least one element is deposited on the surfaces 34 of the metal particles 30 of the metal powder. Heat and pressure is then applied to consolidate the metal particles 30 such that the at least one element of the coating 32 on the surfaces 34 of the metal particles 30 partially diffuses into the metal particles 30 and the coated metal particles 30 are diffusion bonded together to form a cellular structure 36. During the consolidation of the metal particles 30, the roughly spherical metal particles 30 are deformed to a polyhedral shape. This results in a framework of more highly alloyed material 38 located at the boundaries of the diffusion bonded metal particles 30, or adjacent the original surfaces 34 of the metal particles 30. Because there is only limited diffusion of the at least one element from the coating 32 into the metal particles 30, the centres 40 of the consolidated metal particles 30 retain their original composition and thus a cellular structure 36 is created.

The properties of the cellular structure 36 are dependent on the size, diameter, of the metal particles 30 of the metal powder, e.g. the dimensions of the resulting centres 40, and the at least one element in the coating 32. Thus the size, diameter, of the metal particles 30 may be varied to vary the properties of the cellular structure 36 and hence the physical and mechanical properties of the component 10 or 20. The coating 32 for the metal particles 30 may be varied to vary the properties of the cellular structure 36 and hence the physical and mechanical properties of the component 10 or 20.

The coating 32 may comprise an oxide, which is produced by oxidising the surfaces 34 the metal particles 30 in oxygen or air. Alternatively the coating 32 may comprise a nitride, which is produced by nitriding the surfaces 34 of the metal particles 30. Alternatively the coating 32 may comprise a solid solution strengthening element, which is produced by vapour depositing on the surfaces 34 of the metal particles 30. Alternatively the coating 32 may comprise a second metal, having lower melting point than the metal particles 30. Alternatively the coating 32 comprises a second metal powder having a lower yield strength than the metal particles 30. The metal particles 30 may be alloy particles. The second metal may be an alloy. The second metal particles may be alloy particles. The metal particles may be titanium alloy particles. More preferably the titanium alloy particles comprise 6wt% aluminium, 4wt% vanadium and the balance titanium, minor additions and incidental impurities.

The present invention permits modification of the material structure to enhance physical and mechanical properties according to the laws of cellular structures. The present invention produces a cellular structure within a solid metallic component, the cellular structure improves the impact absorption properties, the ductility and the strength of a conventional alloy. In addition physical properties such as the elastic modulus, Poisson's Ratio, friction and damping characteristics are improved.

### Example 1

Titanium alloy particles comprising 6wt% aluminium, 4wt% vanadium and the balance titanium, minor additions and incidental impurities were prepared. The titanium alloy particles were then filtered to the required titanium alloy particle size, 100 micrometers average size and 250 micrometers maximum size. The titanium alloy particles were poured through an inlet tube into and filled a mild steel container, which defines the shape of the component being produced. The container was heated to a temperature of 450°C and maintained at 450°C for 8 hours under a partial air pressure of 10⁻¹ torr to oxidise the titanium alloy particles. The container was then sealed by welding shut an inlet tube. The container was placed in a HIP vessel and hot isostatically pressed at a temperature of 925°C for 2 hours at a pressure of 150MPa. Then the container was removed from the consolidated metal powder component by machining or dissolving in a suitable acid.

The use of a second metal, or second alloy, which has a lower melting point the metal particles will result in melting or evaporation of the second metal to produce a coating on the metal particles. The use of a second metal powder having a lower yield strength than the metal particles will result in the second metal powder deforming around the metal particles during consolidation to produce the cellular structure.

The present invention may also be used to infill metal powder particles into an existing hollow metal structure, for example a hollow fan blade or hollow compressor blade, and then to produce the cellular structure within the existing hollow metal structure. Alternatively, it may be possible to infill metal powder between at least two metal workpieces, then to produce the cellular structure between the at least two metal workpieces and to diffusion bond the cellular structure to the at least two workpieces and to diffusion bond the at least two workpieces together, for example a fan blade.

The present invention may also be used to produce a hollow fan blade of a hollow compressor blade. The mild steel container was provided with one or more removable cores in the mild steel container to define one or more chambers in the hollow fan blade, or hollow compressor blade. The titanium alloy particles were poured into the mild steel container to fill the space in the mild steel container around the one or more removable cores. The container was heated to 450°C and maintained at 450°C for 8 hours under a partial air pressure of 10⁻¹ torr to oxidise the titanium alloy particles. The container was then sealed by welding shut the inlet tube. The container was placed in a HIP vessel and hot isostatically pressed at a temperature of 925°C for 2 hours at a pressure of 150 MPa. Then the container was removed from the consolidated metal powder hollow fan blade, or hollow compressor blade, by machining or dissolving in a suitable acid. Then the removable cores were removed. The removable cores may comprise an inert metal, for example lead or other metal with large atoms which are too large to diffuse into the titanium particles, having a lower melting point than the titanium alloy particles such that the hollow fan blade, or hollow compressor blade, is heated to a temperature at which the inert metal melts and is run out of the hollow fan blade, or hollow compressor blade. Remnants of the metal, may be removed from the hollow fan blade or hollow compressor blade, using a suitable solvent or a suitable acid. The removable cores may comprise mild steel which may be removed with a suitable acid.

Alternatively, the hollow fan blade, or hollow compressor blade may be produced by ensuring that the container defines one or more chambers in the hollow fan blade or hollow compressor blade. The chambers are arranged to be pressurised during the hot isostatic pressing.

The present invention may also entail machining a consolidated metal powder solid fan blade or solid compressor blade to final shape.

The present invention is also applicable to titanium alloy particles comprising 6wt% aluminium, 2wt% tin, 4wt% zirconium, 2wt% molybdenum and the balance titanium, minor additions or incidental impurities.

In the case of oxidising and nitriding the metal particles, or alloy particles, the oxygen or nitrogen partially diffuses into the metal particles, or alloy particles, to form interstitials in the metal, or alloy and the normal, or original, alloy composition at the centres of the consolidated metal particles, or alloy particles, is arranged within a framework of more highly alloyed, interstitial alloy, material located at the boundaries of the diffusion bonded metal particles, or alloy particles.

Although the present invention has been described with reference to titanium alloys, the invention is equally applicable to aluminium alloys, iron alloys, nickel alloys, cobalt alloys and to intermetallics, for example nickel aluminides, titanium aluminides.

## Claims

1. A method of manufacturing a component (10,20) by consolidating a metal powder comprising the steps of:-
(d) preparing a metal powder, the metal powder comprising metal particles (30),
(e) depositing a coating (32) containing at least one element on the surfaces (34) of the metal particles (30) of the metal powder,
(f) applying heat and pressure to consolidate the metal particles (30) such that the at least one element of the coating (32) on the surfaces (34) of the metal particles (30) partially diffuses into the metal particles (30) and the coated metal particles (30) are diffusion bonded together to form a cellular structure (36), the cellular structure (36) comprising a framework of more highly alloyed material (38) located at the boundaries of the diffusion bonded metal particles (30) and the centres (40) of the consolidated metal particles (30) retain their original composition.

2. A method as claimed in claim 1 wherein step (b) comprises oxidising the surfaces (34) of the metal particles (30).

3. A method as claimed in claim 1 wherein step (b) comprises nitriding the surfaces (34) of the metal particles (30).

4. A method as claimed in claim 1 wherein step (b) comprises vapour depositing a solid solution strengthening element on the surfaces (34) of the metal particles (30).

5. A method as claimed in claim 1 wherein step (b) comprises coating the surfaces (34) of the metal particles (30) with a second metal having lower melting point than the metal particles (30).

6. A method as claimed in claim 1 wherein step (b) comprises coating the surfaces (34) of the metal particles (30) with particles of a second metal powder having a lower yield strength than the metal particles (30).

7. A method as claimed in any of claims 1 to 6 wherein the metal particles (30) are alloy particles.

8. A method as claimed in claim 5 wherein the second metal is an alloy.

9. A method as claimed in claim 6 wherein the second metal particles are alloy particles.

10. A method as claimed in claim 7 wherein the metal particles (30) are titanium alloy particles.

11. A method as claimed in claim 10 wherein the titanium alloy particles (30) comprise 6wt% aluminium, 4wt% vanadium and the balance titanium, minor additions and incidental impurities.

12. A method as claimed in claim 11 wherein step a) comprises supplying the titanium alloy particles (30) into a container, step b) comprises oxidising the titanium alloy particles (30), step c) comprises sealing the container and applying heat and pressure.

13. A method as claimed in claim 12 wherein step b) comprises heating to a temperature of 450°C and maintaining at 450°C for 8 hours under a partial pressure of 10⁻¹ torr to oxidise the titanium alloy particles (30) and step c) comprises hot isostatic pressing the container at a temperature of 925°C for 2 hours at a pressure of 150MPa.

14. A method as claimed in claim 12 or claim 13 wherein the container is removed by machining or dissolving in a suitable acid.

15. A method as claimed in claim 12, claim 13 or claim 14 wherein the container comprises mild steel.

16. A method as claimed in any of claims 1 to 15 wherein the metal particles (30) have an average size of 100 micrometers.

17. A method as claimed in any of claims 1 to 16 wherein the metal particles (30) have a maximum size of 250 micrometers.

18. A method as claimed in any of claims 1 to 15 wherein the size of the metal particles (30) is varied to vary the properties of the component (10,20).

19. A component (10,20) comprising consolidated metal powder, the metal powder comprising metal particles (30) diffusion bonded together, the surfaces (34) of the metal particles (30) having a coating having at least one element, which has partially diffused into the metal particles (30) to form a cellular structure (36), the cellular structure (36) comprising a framework of more highly alloyed material (38) located at the boundaries of the diffusion bonded metal particles (30) and the centres (40) of the consolidated metal particles (30) retain their original composition.

20. A component as claimed in claim 19 wherein the coating (34) comprising an oxide or a nitride and the at least one element is oxygen or nitrogen respectively.

21. A component as claimed in claim 19 wherein the coating comprises a solid solution strengthening element on the surfaces of the metal particles (30).

22. A component as claimed in claim 19 wherein the coating (34) comprises a second metal having lower melting point than the metal particles (30).

23. A component as claimed in claim 19 wherein the coating (34) comprises a second metal powder having a lower yield strength than the metal particles (30).

24. A component as claimed in any of claims 19 to 23 wherein the metal particles (30) are titanium alloy particles.

25. A component as claimed in claim 24 wherein the titanium alloy particles (30) comprise 6wt% aluminium, 4wt% vanadium and the balance titanium, minor additions and incidental impurities.

26. A component as claimed in any of claims 19 to 25 wherein the component (10,20) is a gas turbine engine component.

27. A component as claimed in claim 26 wherein the component is a fan blade (20), a part of a fan blade, a compressor blade or a casing (10).

## Patentansprüche

1. Verfahren zur Herstellung eines Bauteils (10, 20) durch Verdichtung eines Metallpulvers mit den folgenden Schritten:
(a) es wird ein Metallpulver vorbereitet, und das Metallpulver weist metallische Partikel (30) auf;
(b) es wird ein Überzug (32), der wenigstens ein Element enthält, auf den Oberflächen (34) der metallischen Partikel (30) des Metallpulvers abgelagert;
(c) es werden Hitze und Druck ausgeübt, um die metallischen Partikel (30) derart zu verdichten, dass das wenigstens eine Element des Überzugs (32) auf den Oberflächen (34) der metallischen Partikel (30) teilweise in die metallischen Partikel (30) hinein diffundiert und die überzogenen metallischen Partikel (30) durch Diffusionsverschweißung miteinander verbunden werden, um eine zellulare Struktur (36) zu erzeugen, wobei die zellulare Struktur (36) einen Rahmen (38) aus höher legiertem Material aufweist, der auf den Grenzflächen der durch Diffusion verbundenen metallischen Partikel (30) angeordnet ist, wobei die Mittelabschnitte (40) der verdichteten metallischen Partikel (30) ihre ursprüngliche Zusammensetzung aufrecht erhalten.

2. Verfahren nach Anspruch 1, bei welchem der Schritt (b) eine Oxidation der Oberflächen (34) der metallischen Partikel (30) umfasst.

3. Verfahren nach Anspruch 1, bei welchem der Schritt (b) eine Nitrierung der Oberflächen (34) der metallischen Partikel (30) umfasst.

4. Verfahren nach Anspruch 1, bei welchem der Schritt (b) eine Dampfablagerung eines Verstärkungselementes einer festen Lösung auf den Oberflächen (34) der metallischen Partikel (30) umfasst.

5. Verfahren nach Anspruch 1, bei welchem der Schritt (b) das Überziehen der Oberflächen (34) der metallischen Partikel (30) mit einem zweiten Metall umfasst, das einen niedrigeren Schmelzpunkt als die metallischen Partikel (30) aufweist.

6. Verfahren nach Anspruch 1, bei welchem der Schritt (b) das Überziehen der Oberflächen (34) der metallischen Partikel (30) mit Partikeln eines zweiten Metallpulvers umfasst, das eine niedrigere Fließfestigkeit als die metallischen Partikel (30) besitzt.

7. Verfahren nach den Ansprüchen 1 bis 6, bei welchem die metallischen Partikel (30) Legierungspartikel sind.

8. Verfahren nach Anspruch 5, bei welchem das zweite Metall eine Legierung ist.

9. Verfahren nach Anspruch 6, bei welchem die zweiten metallischen Partikel Legierungspartikel sind.

10. Verfahren nach Anspruch 7, bei welchem die metallischen Partikel (30) Titan-Legierungspartikel sind.

11. Verfahren nach Anspruch 10, bei welchem die Titan-Legierungspartikel (30) 6 Gewichtsprozent Aluminium, 4 Gewichtsprozent Vanadium und im übrigen Titan, geringe Zusätze und zufällige Verunreinigungen aufweisen.

12. Verfahren nach Anspruch 11, bei welchem der Schritt (a) die Zuführung der Titan-Legierungspartikel (30) in einen Behälter umfasst, und der Schritt (b) eine Oxidation der Titan-Legierungspartikel (30) umfasst, und im Schritt (c) der Behälter abgedichtet und Hitze und Druck ausgesetzt wird.

13. Verfahren nach Anspruch 12, bei welchem der Schritt (b) eine Erhitzung auf eine Temperatur von 450°C umfasst, wobei diese Temperatur von 450°C acht Stunden lang unter einem Partialdruck von 10⁻¹ Torr gehalten wird, um die Titan-Legierungspartikel (30) zu oxidieren, und wobei der Schritt (c) ein heißes, isostatisches Pressen des Behälters bei einer Temperatur von 925°C zwei Stunden lang unter einem Druck von 150 MPa umfasst.

14. Verfahren nach Anspruch 12 oder 13, bei welchem der Behälter durch spanabhebende Bearbeitung oder durch Lösen in einer geeigneten Säure entfernt wird.

15. Verfahren nach Anspruch 12, Anspruch 13 oder Anspruch 14, bei welchem der Behälter aus einem unlegierten Stahl besteht.

16. Verfahren nach einem der Ansprüche 1 bis 15, bei welchem die metallischen Partikel (30) eine durchschnittliche Größe von 100 Mikrometer haben.

17. Verfahren nach einem der Ansprüche 1 bis 16, bei welchem die metallischen Partikel (30) eine maximale Größe von 250 Mikrometer haben.

18. Verfahren nach einem der Ansprüche 1 bis 15, bei welchem die Größe der metallischen Partikel (30) verändert wird, um die Eigenschaften des Bauteils (10, 20) zu verändern.

19. Bauteil (10, 20), bestehend aus einem verdichteten Metallpulver, wobei das Metallpulver metallische Partikel (30) aufweist, die durch Diffusion miteinander verschweißt sind, wobei die Oberflächen (34) der metallischen Partikel (30) einen Überzug aufweisen, der wenigstens ein Element hat, das teilweise in die metallischen Partikel (30) diffundiert ist, um eine zellulare Struktur (36) zu bilden, wobei die zellulare Struktur (36) einen Rahmen aus höher legiertem Material (38) umfasst, der an den Grenzflächen der durch Diffusion verschweißten metallischen Partikel (30) angeordnet ist und die Mittelabschnitte (40) der verdichteten metallischen Partikel (30) ihre ursprüngliche Zusammensetzung aufrecht erhalten.

20. Bauteil nach Anspruch 19, bei welchem der Überzug (34) ein Oxid oder ein Nitrid ist und das wenigstens eine Element Sauerstoff bzw. Stickstoff ist.

21. Bauteil nach Anspruch 19, bei welchem der Überzug ein Verstärkungselement einer festen Lösung auf den Oberflächen der metallischen Partikel (30) aufweist.

22. Bauteil nach Anspruch 19, bei welchem der Überzug (34) ein zweites Metall aufweist, das einen niedrigeren Schmelzpunkt als die metallischen Partikel (30) hat.

23. Bauteil nach Anspruch 19, bei welchem der Überzug (34) ein zweites Metallpulver aufweist, das eine niedrigere Fließfestigkeit hat als die metallischen Partikel (30).

24. Bauteil nach einem der Ansprüche 19 bis 23, bei welchem die metallischen Partikel (30) Titan-Legierungspartikel sind.

25. Bauteil nach Anspruch 24, bei welchem die Titan-Legierungspartikel (30) 6 Gewichtsprozent Aluminium, 4 Gewichtsprozent Vanadium und im übrigen Titan, geringe Zusätze und zufällige Verunreinigungen aufweisen.

26. Bauteil nach einem der Ansprüche 19 bis 25, bei welchem der Bauteil (10, 20) der Bauteil eines Gasturbinentriebwerks ist.

27. Bauteil nach Anspruch 26, bei welchem der Bauteil eine Fan-Laufschaufel (20), ein Teil einer Fan-Laufschaufel, eine Kompressor-Laufschaufel oder ein Gehäuse (10) ist.

## Revendications

1. Procédé pour fabriquer un composant (10, 20) par consolidation de poudre de métal comprenant les étapes de :
(a) préparer une poudre de métal, la poudre de métal comprenant des particules de métal (30),
(b) déposer un revêtement (32) contenant au moins un élément sur les surfaces (34) des particules de métal (30) de la poudre de métal,
(c) appliquer de la chaleur et de la pression pour consolider les particules de métal (30) de sorte que le au moins un élément du revêtement (32) sur les surfaces (34) des particules de métal (30) diffuse partiellement dans les particules de métal (30) et les particules de métal enrobées (30) sont soudées ensemble par diffusion pour former une structure cellulaire (36), la structure cellulaire (36) comprenant une ossature de plusieurs matériaux plus fortement alliés (38) située aux limites des particules de métal soudées par diffusion (30) et les centres (40) des particules de métal consolidées (30) retiennent leur composition d'origine.

2. Procédé selon la revendication 1, dans lequel l'étape (b) comprend d'oxyder les surfaces (34) des particules de métal (30).

3. Procédé selon la revendication 1, dans lequel l'étape (b) comprend de nitrurer les surfaces (34) des particules de métal (30).

4. Procédé selon la revendication 1, dans lequel l'étape (b) comprend de déposer en phase vapeur une solution solide d'élément renforçant sur les surfaces (34) des particules de métal (30).

5. Procédé selon la revendication 1, dans lequel l'étape (b) comprend de revêtir les surfaces (34) des particules de métal (30) avec un deuxième métal ayant un point de fusion inférieur à celui des particules de métal (30).

6. Procédé selon la revendication 1, dans lequel l'étape (b) comprend de revêtir les surfaces (34) des particules de métal (30) avec des particules d'une seconde poudre de métal ayant une limite d'élasticité plus faible que celle des particules de métal (30).

7. Procédé selon l'une quelconque des revendications 1 à 6, dans lequel les particules de métal (30) sont des particules d'alliage.

8. Procédé selon la revendication 5, dans lequel le second métal est un alliage.

9. Procédé selon la revendication 6, dans lequel les secondes particules de métal sont des particules d'alliage.

10. Procédé selon la revendication 7, dans lequel les particules de métal (30) sont des particules d'alliage de titane.

11. Procédé selon la revendication 10, dans lequel les particules d'alliage de titane (30) comprennent 6% en poids d'aluminium, 4% en poids de vanadium et le reste en titane, des ajouts et impuretés accidentelles mineures.

12. Procédé selon la revendication 11, dans lequel l'étape (a) comprend de fournir des particules d'alliage de titane (30) dans un conteneur, l'étape (b) comprend d'oxyder les particules d'alliages de titane (30), l'étape (c) comprend de sceller le conteneur et d'appliquer de la chaleur et de la pression.

13. Procédé selon la revendication 12, dans lequel l'étape (b) comprend de chauffer à une température de 450°C et maintenir à 450°C pendant huit heures sous une pression partielle de 10⁻¹ torr pour oxyder les particules d'alliages de titane (30) et l'étape (c) comprend de presser de manière isostatique à chaud le conteneur à une température de 925°C pendant deux heures à une pression de 150 MPa.

14. Procédé selon la revendication 12 ou la revendication 13, dans lequel le conteneur est retiré par usinage ou dissolution dans un acide approprié.

15. Procédé selon la revendication 12, 13 ou 14, dans lequel le conteneur comprend un acier doux.

16. Procédé selon l'une quelconque des revendications 1 à 15, dans lequel les particules de métal (30) ont une taille moyenne de 100 micromètres.

17. Procédé selon l'une quelconque des revendications 1 à 16, dans lequel les particules de métal (30) ont une taille maximale de 250 micromètres.

18. Procédé selon l'une quelconque des revendications 1 à 15, dans lequel la taille des particules de métal (30) est variée pour modifier les propriétés du composant (10, 20).

19. Composant (10, 20) comprenant de la poudre de métal consolidée, la poudre de métal comprenant des particules de métal (30) soudées ensemble par diffusion, les surfaces (34) des particules de métal (30) ayant un revêtement qui a au moins un élément, qui a partiellement diffusé dans les particules de métal (30) pour former une structure cellulaire (36), la structure cellulaire (36) comprenant une ossature de matériau (38) plus fortement allié situé aux limites des particules de métal (30) soudées par diffusion et les centres (40) des particules de métal consolidées (30) conservent leur composition d'origine.

20. Composant selon la revendication 19, dans lequel le revêtement (34) comprend un oxyde ou un nitrure et le au moins un élément est respectivement de l'oxygène ou de l'azote.

21. Composant selon la revendication 19, dans lequel le revêtement comprend une solution solide d'élément renforçant sur les surfaces des particules de métal (30).

22. Composant selon la revendication 19, dans lequel le revêtement (34) comprend un second métal ayant un point de fusion inférieur à celui des particules de métal (30).

23. Composant selon la revendication 19, dans lequel le revêtement (34) comprend une seconde poudre de métal ayant une limite d'élasticité inférieure à celles des particules de métal (30).

24. Composant selon l'une quelconque des revendications 19 à 23, dans lequel les particules de métal (30) sont des particules d'alliage de titane.

25. Composant selon la revendication 24, dans lequel les particules d'alliage de titane (30) comprennent 6% en poids d'aluminium, 4% en poids de vanadium et le reste en titane, des ajouts et impuretés accidentelles mineures.

26. Composant selon l'une quelconque des revendications 19 à 25, dans lequel le composant (10, 20) est un composant de moteur de turbine à gaz.

27. Composant selon la revendication 26, dans lequel le composant est une pale de soufflante (20), une partie d'une pale de soufflante, une pale de compresseur ou un carter (10).
